

## 1

3,746,767

**MOTHPROOFING WOOL**

Anthony M. Schwartz, Rockville, and Charles A. Rader, Laurel, Md., assignors to the United States of America as represented by the Secretary of Agriculture  
 No Drawing. Filed Jan. 7, 1971, Ser. No. 104,762  
 Int. Cl. A01n 9/20

U.S. Cl. 424—329

7 Claims

**ABSTRACT OF THE DISCLOSURE**

A very limited group of quaternary ammonium compounds were found to effectively mothproof wool. Tricaprylylmethylammonium chloride (Aliquat 336), diacyldimethylammonium chloride (Aliquat 203), and dioctyldimethylammonium chloride (Aliquat 202) at add-on levels as low as 0.5% provided very good protection against both black carpet beetle and webbing clothes moth larval feeding.

A non-exclusive, irrevocable, royalty-free license in the invention herein described, throughout the world for all purposes of the United States Government, with the power to grant sublicenses for such purposes, is hereby granted to the Government of the United States of America.

This invention relates to the treatment of wool and other animal hair and keratinous material to render it resistant to attack by moths. More particularly, it relates to the treatment of wool with a certain very limited class of quaternary ammonium compounds to impart durable moth-resistant properties without introducing toxicity or other hazardous or disadvantageous effects to the wool.

The art of mothproofing wool is old and extensive. The most widely used chemical method is to impregnate wool with a compound that discourages the moth larvae from eating, either by being distasteful and therefore repellent or by being toxic. A great variety of compound representing many chemical types have been described as mothproofers in both the patent and the journal literature. Among these compounds are several of the long chain quaternary ammonium type. However, none, to our knowledge, has the specific structural features and correspondingly advantageous performance characteristics of the compounds used in the present invention.

In order to determine the efficacy of a method of treating wool to render it mothproof or to determine the efficacy of a compound or other substance as a mothproofing agent, the results obtained with the method or performance of the compound as a mothproofing agent must be considered.

The following are the performance requirements that should be considered in the determination of the mothproofing efficacy of a method or a compound.

(1) It must effectively protect the wool from larval attack when present in relatively small amounts, generally less than 2.0% relative to the weight of wool. The effectiveness is tested by exposing the wool, under well-controlled conditions, to the larvae for a specified time. Damage is estimated by weight loss, by weight of larval excrement, and by visual inspection.

(2) It must not alter the handle, color or other functional properties of the wool.

(3) It must not be toxic, and must not cause dermatitis, itching, etc., to the user of the woolen garment or goods.

(4) It must remain on the goods and be effective when subjected to multiple washings and drycleanings.

(5) It must be easy to apply to the goods, either during or after fabrication, by processes that do not matt or shrink or otherwise alter the desirable characteristics of the wool.

## 2

The more successful of the quaternary ammonium types previously used for mothproofing have adequately met requirements 2 and 3 above, and to a certain extent requirement 5. Requirements 1 and 4, effectiveness and durability, have not, however, been adequately satisfied. The best compounds to date, and their performance characteristics, are described by Freeland and Williams, Textile Research Journal 37, 408–416 (1967). All of them are characterized by having a single long chain alkyl group on the quaternary nitrogen atom. The chain length of this group is in the usual surfactant range, that is 12–18 carbon atoms. The remaining groups on the nitrogen are the usual nonsurface active lower alkyl pyridyl or benzyl, and together they take up the three valencies on the nitrogen other than that taken up by the long chain alkyl group.

It is an object of this invention to provide mothproofing agents that exhibit all of the above listed desirable performance requirements.

Another object of this invention is to provide a method of treating wool which will render the wool mothproof.

In general, according to this invention, wool is made mothproof by treating it with a quaternary ammonium compound of one of the following general formulas

 25  
 30


wherein R, R' and R'' are straight chain alkyl groups of 8 to 10 carbon atoms, a and b are alkyl groups of 1 to 3 carbon atoms, X<sup>-</sup> is an anion such as Cl<sup>-</sup>, Br<sup>-</sup>, SO<sub>4</sub>CH<sub>3</sub><sup>-</sup>, and SO<sub>4</sub>C<sub>2</sub>H<sub>5</sub><sup>-</sup>, that together with the nitrogenous cation forms a soluble salt. This treatment combines all the desirable properties of a mothproofing agent including exceptional durability to washing and drycleaning and effectiveness in low concentrations of the selected compound.

The compounds of this invention are soluble in water and may be applied to woolen goods by padding, soaking, or spraying. The effects of temperature, pH, and inorganic salts in the bath and the extent and rate of take-up are those expected when a typical cationic surfactant is applied to wool. The compounds of this invention, however, combine unexpectedly high toxicity to moth larvae with high resistance to removal by laundering or drycleaning. In addition, solutions of the compounds in non-aqueous solvents may also be used to treat the wool.

The following examples demonstrate the application of the process:

**EXAMPLE 1**

Application to woven woolen piece goods by padding

Eight by twelve inch swatches of clean wool flannel were treated in a conventional padding machine with a 0.3% solution of tricaprylylmethylammonium chloride (Aliquat 336) in which the three caprylyl groups are a mixture of C<sub>8</sub> and C<sub>10</sub>. The treating bath also contained .01% of Tergitol NPX the monoether of nonyl phenol with a polyethylene glycol mixture having an average chain length of 10.5 ethylene oxide (a nonionic surfactant) that served as a wetting agent. The pad roll pressure was 20 p.s.i., providing a wet pick-up of 108%. After drying, the add-on of quaternary compound was measured at 0.32% on the weight of wool. The material thus treated was resistant to the attack of black carpet beetle larvae and webbing clothes moth larvae when tested by the C.S.M.A. (Chemical Specialties Manufacturer's Association) and A.A.T.C.C. (American Association of Textile Chemists and Colorists) test methods.

## EXAMPLE 2

## Application by soaking

Raw wool was scoured in a conventional scouring procedure, except that the last rinse bowl, instead of containing water contained a .01% solution of didecyldimethylammonium chloride (Aliquat 203). The wool was left in this bath for 4 minutes. The add-on was determined after squeezing and drying in the conventional manner, and was 0.7%. This material was resistant to moth larvae and retained its resistance through all subsequent manufacturing steps to the final woven fabric. Tables I-II show the results obtained by immersing accurately weighed wool swatches in aqueous quaternary salt solutions. Table I shows the percent depletion of the bath and the percent add-on of quaternary salt on the wool. Tables II and III show the resistance of quaternary treated wool to black carpet beetle larvae and to webbing clothes moth larvae respectively. Add-on levels as low as 0.5% provided very good protection against both black carpet beetle and webbing clothes moth larvae feeding.

Minimum effective levels of the quaternary salts as insect deterrents were determined using tricaprylylmethylammonium chloride (Aliquat 336) as the mothproofing agent. Accurately weighed wool swatches were immersed and agitated in aqueous solutions of the quaternary in a borax buffer of pH 9.2. The wool-liquor ratio was 1:20. The treatment was done at 38-40° C. for two hours. Concentration of the quaternary bath was determined before and after the adsorption treatment, percent depletion of the bath and percent add-on of quaternary on the wool calculated, and effectiveness of the treatment against black carpet beetle larvae and webbing clothes moth larvae determined. The data are shown in Tables IV to VI.

The data of Table V show that the treated wool containing the 0.25% and 0.50% quaternary add-on were satisfactorily protected against black carpet beetle larvae feeding. The treated wool containing 0.10% quaternary add-on just failed with 0.52 mg. excrement (0.50 mg. or less in passing). However, as shown in Table VI, treated wool containing 0.10% and higher quaternary add-on levels were protected from webbing clothes moth larvae.

As shown in Tables VII and VIII, even at add-on levels as low as 0.15%, the quaternary salt retained its effectiveness during storage against both black carpet beetle and webbing clothes moth larvae feeding. As shown by the excrement weights per larva and the adjusted weight losses, wool swatches treated with tricaprylylmethylammonium chloride and aged for periods up to nine months were satisfactorily protected at 0.15 to 0.50% add-on levels.

TABLE II.—RESISTANCE OF QUATERNARY AMMONIUM HALIDE TREATED WOOL TO BLACK CARPET BEETLE LARVAE

|    | Quaternary add-on, percent                            | Excrement per larva, mg. | Mortality, percent |
|----|-------------------------------------------------------|--------------------------|--------------------|
| 5  | Dioctyldimethylammonium chloride (Aliquat 202).....   | 0.4                      | 0.42               |
|    | .....                                                 | 1.0                      | 0.25               |
|    | .....                                                 | 2.0                      | 0.30               |
|    | .....                                                 | 2.6                      | 0.25               |
|    | .....                                                 | 3.4                      | 0.21               |
| 10 | Untreated check.....                                  | 2.19                     | 0                  |
| 15 | Tricaprylylmethylammonium chloride (Aliquat 336)..... | 0.5                      | 0.28               |
|    | .....                                                 | 1.0                      | 0.25               |
|    | .....                                                 | 2.0                      | 0.25               |
|    | .....                                                 | 3.0                      | 0.21               |
|    | .....                                                 | 4.0                      | 0.23               |
| 20 | Untreated check.....                                  | 1.91                     | 0                  |
| 25 | Didecyldimethylammonium chloride (Aliquat 203).....   | 0.5                      | 0.28               |
|    | .....                                                 | 1.0                      | 0.26               |
|    | .....                                                 | 2.0                      | 0.27               |
|    | .....                                                 | 2.9                      | 0.25               |
|    | Untreated check.....                                  | 2.19                     | 0                  |

NOTE.—The fabric is considered satisfactorily resistant to black carpet beetle larvae if the average quantity of excrement per larva is not over 0.5 mg. provided that no single value is over 0.6 mg., and the untreated check is over 1.5 mg.

TABLE III.—RESISTANCE OF QUATERNARY AMMONIUM HALIDE TREATED WOOL TO WEBBING CLOTHES MOTH LARVAE

|    | Quaternary add-on, percent                            | Adjusted weight loss, mg. | Mortality, percent |
|----|-------------------------------------------------------|---------------------------|--------------------|
| 30 | Dioctyldimethylammonium chloride (Aliquat 202).....   | 0.4                       | 7.71               |
|    | .....                                                 | 1.0                       | 4.28               |
|    | .....                                                 | 2.0                       | 3.58               |
|    | .....                                                 | 2.6                       | 3.41               |
|    | .....                                                 | 3.4                       | 2.77               |
| 35 | Untreated check.....                                  | 31.46                     | 12.5               |
| 40 | Tricaprylylmethylammonium chloride (Aliquat 336)..... | 0.5                       | 5.47               |
|    | .....                                                 | 1.0                       | 3.82               |
|    | .....                                                 | 2.0                       | 1.63               |
|    | .....                                                 | 3.0                       | 1.34               |
|    | .....                                                 | 4.0                       | 2.18               |
| 45 | Untreated check.....                                  | 36.63                     | 17.5               |
| 50 | Didecyldimethylammonium chloride (Aliquat 203).....   | 0.5                       | 5.82               |
|    | .....                                                 | 1.0                       | 3.69               |
|    | .....                                                 | 2.0                       | 0.93               |
|    | .....                                                 | 2.9                       | 1.45               |
|    | Untreated check.....                                  | 31.46                     | 12.5               |

NOTE.—Fabric is considered satisfactorily resistant to webbing clothes moth larvae if the average weight loss due to feeding is not more than 8 mg.; provided the weight loss of no individual sample is more than 10 mg. The weight loss of the untreated check should be 30 mg. or more.

TABLE I.—ADSORPTION OF QUATERNARY AMMONIUM HALIDES ONTO WOOL

| Compound                                              | Initial concentration of the quaternary bath, percent active ingredient | Temperature of adsorption treatment, °C. | Time of adsorption treatment, hours | Exhaust of bath, percent | Quaternary add-on, on wool, percent |
|-------------------------------------------------------|-------------------------------------------------------------------------|------------------------------------------|-------------------------------------|--------------------------|-------------------------------------|
| Dioctyldimethylammonium chloride (Aliquat 202).....   | 0.020                                                                   | 38-40                                    | 2                                   | 100.0                    | 0.4                                 |
|                                                       | 0.050                                                                   | 38-40                                    | 2                                   | 98.0                     | 1.0                                 |
|                                                       | 0.100                                                                   | 38-40                                    | 2                                   | 98                       | 2.0                                 |
|                                                       | 0.150                                                                   | 38-40                                    | 2                                   | 87                       | 2.6                                 |
|                                                       | 0.200                                                                   | 38-40                                    | 2                                   | 84                       | 3.4                                 |
| Tricaprylylmethylammonium chloride (Aliquat 336)..... | 0.200                                                                   | 35-37                                    | 2                                   | 98.8                     | 4.0                                 |
|                                                       | 0.150                                                                   | 35-37                                    | 2                                   | 100                      | 3.0                                 |
|                                                       | 0.100                                                                   | 35-37                                    | 2                                   | 100                      | 2.0                                 |
|                                                       | 0.050                                                                   | 35-37                                    | 2                                   | 100                      | 1.0                                 |
|                                                       | 0.025                                                                   | 35-37                                    | 2                                   | 100                      | 0.5                                 |
| Didecyldimethylammonium chloride (Aliquat 203).....   | 0.025                                                                   | 38-40                                    | 2                                   | 100                      | 0.5                                 |
|                                                       | 0.050                                                                   | 38-40                                    | 2                                   | 100                      | 1.0                                 |
|                                                       | 0.100                                                                   | 38-40                                    | 2                                   | 100                      | 2.0                                 |
|                                                       | 0.150                                                                   | 38-40                                    | 2                                   | 98                       | 2.9                                 |
|                                                       | 0.200                                                                   | 38-40                                    | 2                                   | 99                       | 3.9                                 |

TABLE IV

| Compound                                            | Initial concentration of quaternary bath (percent) | Exhaust of bath, percent | Quaternary add-on, percent |
|-----------------------------------------------------|----------------------------------------------------|--------------------------|----------------------------|
| Tricaprylylmethylammonium chloride (Aliquat 336) .. | 0.0025                                             | 100                      | 0.05                       |
|                                                     | 0.0050                                             | 100                      | 0.10                       |
|                                                     | 0.0125                                             | 100                      | 0.25                       |
|                                                     | 0.0250                                             | 100                      | 0.50                       |

TABLE V

| Compound                                            | Add-on, percent | Excrement per larva, mg. | Mortality, percent |
|-----------------------------------------------------|-----------------|--------------------------|--------------------|
| Tricaprylylmethylammonium chloride (Aliquat 336) .. | 0.05            | 0.72                     | 0                  |
|                                                     | 0.10            | 0.52                     | 0                  |
|                                                     | 0.25            | 0.31                     | 0                  |
|                                                     | 0.50            | 0.30                     | 0                  |
| None: Untreated check ..                            |                 | 1.75                     | 0                  |

TABLE VI

| Compound                                            | Add-on, percent | Adjusted weight loss, mg. | Mortality, percent |
|-----------------------------------------------------|-----------------|---------------------------|--------------------|
| Tricaprylylmethylammonium chloride (Aliquat 336) .. | 0.05            | 10.00                     | 73                 |
|                                                     | 0.10            | 5.58                      | 70                 |
|                                                     | 0.25            | 2.86                      | 80                 |
|                                                     | 0.50            | 1.89                      | 92                 |
| None: Untreated check ..                            |                 | 36.26                     | 12                 |

TABLE VII.—EFFECTIVENESS OF MOTHPROOFING AGENT AGAINST BLACK CARPET BETTLE LARVAE DURING STORAGE

| Compound                                            | Add-on, percent | Excrement per larva, mg. |               |                |                |                |
|-----------------------------------------------------|-----------------|--------------------------|---------------|----------------|----------------|----------------|
|                                                     |                 | Initial test             | 1-month aging | 2-months aging | 3-months aging | 9-months aging |
| Tricaprylylmethylammonium chloride (Aliquat 336) .. | 0.15            | 0.39                     | 0.29          | 0.39           | 0.35           | 0.30           |
|                                                     | 0.25            | 0.31                     | 0.30          | 0.32           | 0.34           | 0.26           |
|                                                     | 0.50            | 0.24                     | 0.28          | 0.29           | 0.28           | 0.28           |
| None: Untreated check ..                            |                 | 2.10                     | 1.90          | 1.62           | 1.73           | 2.00           |

TABLE VIII.—EFFECTIVENESS OF MOTHPROOFING AGENT AGAINST WEBBING CLOTHES MOTH LARVAE DURING STORAGE

| Quaternary compound                                 | Add-on, percent | Adjusted weight loss of wool, mg. <sup>a</sup> |              |               |               |               |
|-----------------------------------------------------|-----------------|------------------------------------------------|--------------|---------------|---------------|---------------|
|                                                     |                 | Initial                                        | Aged 1-month | Aged 2-months | Aged 3-months | Aged 9-months |
| Tricaprylylmethylammonium chloride (Aliquat 336) .. | 0.15            | 4.92                                           | 5.00         | 7.27          | 6.31          | 5.97          |
|                                                     | 0.25            | 2.29                                           | 3.89         | 5.61          | 3.77          | 4.49          |
|                                                     | 0.50            | 1.33                                           | 3.65         | 2.14          | 3.30          | 1.72          |
| None: Untreated wool ..                             |                 | 41.32                                          | 54.84        | 43.60         | 33.19         | 35.00         |

<sup>a</sup> Moth larvae mortalities were also determined. Mortality was 70-100% for the various Aliquat-treated samples and 7-17% for the untreated wool.

We claim:

1. A process of mothproofing wool consisting of treating the wool with a quaternary ammonium compound having a formula selected from the group consisting of



and



wherein R, R' and R'' are selected from the group consisting of straight chain alkyls containing from 8 to 10 carbons, a and b are methyl, X<sup>-</sup> is an anion selected from the group consisting of Cl<sup>-</sup>, Br<sup>-</sup>, SO<sub>4</sub>CH<sub>3</sub><sup>-</sup>, and SO<sub>4</sub>C<sub>2</sub>H<sub>5</sub><sup>-</sup>, said treatment adding to the wool an effective amount of at least 0.15% of an aforesaid quaternary ammonium compound.

2. The process of claim 1 wherein R, R' and R'' are alkyls containing 8 carbons and X<sup>-</sup> is Cl<sup>-</sup>.

3. The process of claim 1 wherein R and R' are alkyls containing 8 carbons and X<sup>-</sup> is Cl<sup>-</sup>.

4. The process of claim 1 wherein R and R' are alkyls containing 10 carbons and X<sup>-</sup> is Cl<sup>-</sup>.

5. The process of claim 1 wherein the quaternary ammonium compound is applied by padding the wool with an aqueous solution of said compound.

6. The process of claim 1 wherein the quaternary ammonium compound is applied by immersing the wool in a solution of said compound.

7. A process for treating wool to make the wool resistant to the larval feeding of the black carpet beetle and the webbing clothes moth consisting of immersing and agitating the wool in an aqueous solution containing an effective amount of at least 0.005% of a quaternary ammonium compound selected from the group consisting of tri(octyl-decyl)methylammonium chloride, dioctyldimethylammonium chloride, and didecyldimethylammonium chloride, said aqueous solution containing a borax buffer of pH 9.2 and said treatment being done at 38 to 40° C. for 2 hours.

6

#### References Cited

##### UNITED STATES PATENTS

- 3,033,704 5/1962 Sherrill et al. ----- 117—138.5  
 3,058,881 10/1962 Wilde ----- 117—138.5 X  
 3,247,058 4/1966 Hyman ----- 117—138.5 X

##### OTHER REFERENCES

- 60 Freeland et al.: Textile Research Journal, vol. 37, pp. 408-16, May 1967.  
 McCutcheon's Detergents and Emulsifiers 1969 Annual, p. 42.  
 65 Tolgyesi et al.: Chem. Tech., pp. 27-30, January 1971.

STANLEY J. FRIEDMAN, Primary Examiner

U.S. Cl. X.R.

117—138.5